# EUROPEAN PATENT SPECIFICATION

(11) **EP 0 939 345 B1**
(45) Date of publication and mention of the grant of the patent: **20.07.2005**
(21) Application number: 99301453.9
(22) Date of filing: 26.02.1999
(51) Int. Cl.: G03G 9/08, G03G 9/097

(54) **Toner composition and method of preparing toner using the same**
Tonerzusammensetzung und deren Herstellung
Composition de révélateur et procédé pour sa préparation

(30) Priority: 27.02.1998 KR 9806468
(43) Date of publication of application: 01.09.1999
(73) Proprietor: SAMSUNG ELECTRONICS CO., LTD., Suwon-City, Kyungki-do (KR)
(72) Inventor: Park, Moon-soo, Dongjak-gu, Seoul (KR); Hong, Soon-kil, Suwon-city, Kyungki-do (KR); Noh, Jin-young, Kwangmyung-city, Kyungki-do (KR)
(74) Representative: Chugg, David John

(56) References cited:
- EP-A- 0 230 041
- EP-A- 0 371 811
- EP-A- 0 376 343
- DE-A- 4 202 462
- PATENT ABSTRACTS OF JAPAN vol. 13, no. 57 (P-825), 9 February 1989 & JP 63 247760 A (CANON), 14 October 1988

## Description

The present invention relates to a toner composition and a method of preparing toner using the same, and more particularly, to a toner composition having improved particle diameter and charge quantity characteristics of toner as well as improved dispersion property of a colouring agent, and a method of preparing toner using the toner composition.

Recently, demand for printers has gradually increased with development in computer industries. Accordingly, the amount of toner used has also increased.

Toner particles used for displaying an image are generally prepared by a grinding method. According to the grinding method, a polymer bonding resin, a colouring agent and a charge controller, etc. are blended in a dry condition. Then, the mixture is melt-mixed and cooled. The resultant is ground to fine toner particles.

Toner particles prepared by the above method have a wide distribution of particle diameters. Because toner particles outside a predetermined diameter range must be excluded, it is an economically unfavourable method. Limitation in dispersion of the charge controller and the colouring agent, and the shape of the toner particles often leads to an unsatisfactory resolution. To solve these problems, spherical toner particles have been prepared by polymerization technique.

This polymerization technique is classified into an emulsion polymerization method and a suspension polymerization method. According to the emulsion polymerization method, the final toner particle is usually smaller than 5µm in diameter. It, however, causes an adverse effect on human body. As a result, it would be is difficult to use these particles in preferred printers. This is why the suspension polymerization method is a preferred polymerization method.

A method of preparing toner by the suspension polymerization method is described as follows.

Water is used as a reaction medium, and a monomer for a binding resin, a charge controller, a stabilizer, a lubricant and a colouring agent are added to the reaction medium, and then polymerization is performed.

After the polymerization is completed, spherical particles sediment inside the reaction mixture. The obtained particles are filtered and then dried, producing the toner particles.

Phosphate or hydrophobic silica is used as the stabilizer. When using phosphate as the stabilizer, however, the particle diameter of the final toner particles tends to be very large, i.e., over approximately 35µm, and the particle diameter distribution shows a wide variation ranging from a few to hundred micrometers in diameter. These particles contributes to lowering charge characteristics, and thus not have proper properties as toner.

On the other hand, when the hydrophobic silica is used as the stabilizer, it is very difficult for the silica to be dispersed into the water. As a result, the polymerization reaction cannot occur. Therefore, the hydrophobic silica must be solubilized in an organic solvent, such as methanol, before it could be miscible with the other constituents of the toner composition for the polymerization.

To solve the above problems, it is an aim of preferred embodiments of the present invention to provide a toner composition which has improved particle diameter characteristics of toner particles and dispersion properties of filler particles, such as a charge controller and a colouring agent.

DE 42 02 462 A relates to a toner polymerizable composition comprising a polymerizable monomer, a colouring agent, 0 to 10 parts charge control substances, 0 to 10 parts antioffset agent is added to an amorphous silicon dioxide dispersion at pH 9 to 14, the pH of the resultant mixture is reduced to pH 2 to 7 and polymerization performed at this pH range.

EP-A-0 371 811 discloses the use of an ionic surface active agent in a toner polymerization composition containing a dispersant, a monomer, a polymerization initiator. The pH of the solution is varied to dissolve and précipitate the dispersant.

It is another aim of preferred embodiments of the present invention to provide a method of preparing toner using the composition.

According to a first aspect of the invention, there is provided a toner polymerizable composition comprising a monomer for a binding resin, a colouring agent, a charge controller, a lubricant, a polymerization initiator, a stabilizer obtained by dispersing hydrophobic silica into distilled water of pH 10-14, and then adjusting the pH of the dispersion into the range 6-8, and an ionic surfactant, and wherein the mixing ratio of the monomer for binding resin and the ionic surfactant is between 1000:1 and 2000:1 by weight.

Preferably, the mixing ratio of the monomer for a binding resin and the silica solid content is between 50:1 and 25:1 by weight.

The ionic surfactant is preferably selected from the group consisting of sodium lauryl sulfate, cetyltrimethylammonium bromide and cetyltrimethylammonium chloride.

According to a second aspect of the invention, there is provided a method of preparing a toner composition comprising the steps of:
(a) adjusting the pH of distilled water to pH 10-14 with an aqueous base, and dispersing hydrophilic silica into the pH-adjusted distilled water;
(b) adjusting the pH of the mixture of the step (a) to pH 6-8;
(c) mixing a monomer for a binding resin, a polymerization initiator, a charge controller, a lubricant, a colouring agent, and an ionic surfactant, and adding the mixture to the resultant of the step (b);
(d) preparing toner particles by polymerizing the resultant of the step (c); and
(e) removing foreign materials remaining on the surface of toner particles;
wherein the mixing ratio of the monomer for binding resin and the ionic surfactant is between 1000:1 and 2000:1 by weight.

By "distilled water" we mean any water of high purity, including demineralised or de-ionised water, or any other purified grade of water.

Preferably, the aqueous base is selected from the group consisting of ammonium hydroxide, sodium hydroxide and potassium hydroxide.

The mixing ratio of the monomer for a binding resin and the silica solid content is preferably between 50:1 and 25:1 by weight.

Preferably, the ionic surfactant is selected from the group consisting of sodium lauryl sulfate, cetyltrimethylammonium bromide and cetyltrimethylammonium chloride.

For a better understanding of the invention, and to show how embodiments of the same may be carried into effect, reference will now be made, by way of example, to the accompanying diagrammatic drawings, in which:
Figures 1 through 5 show representations of optical microscope photographs of toner particles prepared by Example 1 (Figure 3) according to embodiments of the present invention and Comparative Examples 1, 2, 5 and 6; and
Figures 6 through 10 are diagrams showing distribution of particle diameter of toner particles prepared by Example 1 (Figure 8) according to the embodiments of the present invention and Comparative Examples 1, 2, 5 and 6.

A toner composition of an embodiment of the present invention is characterized by a stabilizer which is obtained by dissolving hydrophobic silica in distilled water of pH 10-14, and then neutralizing the resultant to pH 6-8. When thus-obtained stabilizer is mixed with a monomer for a binding resin, a colouring agent, a charge controller, an ionic surfactant, a lubricant and a polymerization initiator, a uniformly dispersed toner composition can be obtained unlike the conventional toner composition.

Preferably, the mixing ratio of the monomer for a binding resin and the silica solid content is between 50:1 and 25:1 by weight. Here, if the mixing content of the silica solid is over the above range, it is very difficult to recover toner particles after polymerization. Also, if the mixing content of the silica solid is less than the above range, toner particles agglomerate unfavourably.

Here, the ionic surfactant may be an anionic or cationic surfactant without restriction.

As the anionic surfactant, sodium lauryl sulfate is suitably used. The cationic surfactant may be cetyltrimethylammonium bromide or cetyltrimethylammonium chloride. Also the mixing ratio between the monomer for a binding resin and the surfactant is in the range of 1000:1-2000:1 by weight. Here, if the mixing content of the surfactant exceeds the above range, it is difficult to recover toner particles. On the other hand, if the mixing content of the surfactant is less than the above range, dispersion properties of filler particles become poor.

The monomer for a binding resin includes any monomers generally used when preparing toner particles by polymerization. In the present invention, a combination of styrene and butylmethacrylate is preferably used. Here, the mixing ratio of styrene and butylmethacrylate is suitably 6:4-9:1 based on weight, preferably 7:3-8:2.

The charge controller controls the charging properties of the toner, and includes any general charge controllers without limitations. Also, the colouring agent is suitably carbon black as a black pigment.

The lubricant improves fluidity of toner particles. Here, wax is suitably used for this purpose. Also, the polymerization initiator may be any general polymerization initiator.

Hereinafter, a method of preparing toner particles using the toner composition will be described.

After adjusting the pH of distilled water to 10-14 using an aqueous base, hydrophobic silica is dispersed into the pH-adjusted distilled water. Then, the mixture is neutralized to pH 6-8. Here, the aqueous base may be sodium hydroxide, potassium hydroxide or ammonium hydroxide without limitation. Also, so as to neutralize the hydrophobic silica dispersion of pH 10-14, any acid may be used without restriction. However, formic acid is preferred.

A mixture of a monomer for a binding resin, a charge controller, a colouring agent, a lubricant, an ionic surfactant and a polymerization initiator is added to the resultant, and then uniformly mixed. Preferably the ionic surfactant, is an cationic surfactant. This mixing process is preferably performed by a ball mill.

Then, polymerization is performed on the resultant under an inert atmosphere, for example nitrogen. After the polymerization is completed, unreacted residues are removed from the reaction mixture using methanol. Here, if a conversion ratio of the polymerization reaction reaches as low as 70-80%, then methanol is preferably used to remove the unreacted residues. On the other hand, if the conversion is found to be as high as 80% or over, the unreacted residues are preferably removed using distilled water.

Then, the obtained precipitate is filtered, and foreign materials remaining on the surface of the precipitate are removed using a dilute potassium hydroxide aqueous solution or methanol. The resultant mass from which the foreign materials were removed is dried in a vacuum oven for a predetermined time, thereby resulting in toner particles of the present invention.

The average diameter of the toner particles obtained by the above method is 5~20µm, the charge quantity is -10~-20µc/g, and the glass transition temperature is 60-75°C.

Hereinafter, embodiments of the present invention will be described through the following examples. However, the present invention is not limited to the following examples.

### Comparative Example 1.

Ammonium hydroxide aqueous solution was added to 600ml of distilled water to adjust the pH to approximately 10, and then 6g of hydrophobic silica S-972 (Degussa Co.) was added to the pH-adjusted distilled water. Then, the resultant was stirred using a homogenizer at 5,000rpm for 10 minutes. Then, the resultant was neutralized using formic acid to prepare a first composition.

140ml of styrene, 60ml of butylmethacrylate, 4g of 2,2-azobisisobutyronitrile, 6g of Carbon black 2350 (Mitsubishi Co., average diameter: 15nm), 2g of Bontron S-34 (Orient Chemical Co.) and 2g of wax were mixed to prepare a second composition.

The mixture of the first composition and the second composition was stirred in a ball-mill for 12 hours. Then, the polymerization was performed at 75°C for 7 hours under a nitrogen atmosphere.

After the polymerization was completed, unreacted styrene and butylmethacrylate were removed from the reaction mixture using methanol. Then, the resultant was filtered and cleaned, and dried in a vacuum oven for 2 days, resulting in toner particles.

### Comparative Example 2

Toner particles were prepared by the same method as Example 1, except that the carbon black content was 10g.

### <Example 1>

Toner particles were prepared by the same method as Comparative Example 1, except that 0.1g of cetyltrimethylammonium bromide (CTAB) was additionally included in the first composition.

### <Comparative Example 3>

400ml of distilled water and 100ml of methanol were mixed, and then 6g of hydrophobic silica R-972 (Degussa Co.) was dispersed into the mixture, to prepare a first composition.

140ml of styrene and 60ml of butylmethacrylate were mixed with 600ml of distilled water, and then 4g of 2,2-azobisisobutyronitrile, 6g of carbon black, 2g of Bontron S-34 and 2g of wax were added to the mixture, to prepare a second composition.

After adding the second composition to the first composition, the polymerization was performed on the reaction mixture at 75°C for 7 hours under a nitrogen atmosphere.

After the reaction was completed, unreacted styrene and butylmethacrylate were removed from the reaction mixture using methanol. Then, the resultant was filtered and cleaned, and then dried in a vacuum oven for 2 days, resulting in toner particles.

### <Comparative Example 4>

Toner particles were prepared by the same method as Example 1, except that di-n-butylamine was used to prepare the first composition instead of ammonium hydroxide aqueous solution.

### <Comparative Example 5>

3g of tri-calcium phosphate (Ca₃(PO₄)₂, Yakuri Pure Chemicals) was added to 600ml of distilled water, to prepare a first composition.

140ml of styrene, 60ml of butylmethacrylate, 2g of 2,2-azobisisobutyronitrile, 6g of Carbon black 2350 (Mitsubishi Co., average diameter: 15nm), 2g of Bontron S-34 (Orient Chemical Co.) and 2g of wax were mixed to prepare a second composition.

After adding the second composition to the first composition, the mixture was stirred in a ball-mill for 12 hours. Then, the polymerization was performed at 75°C for 7 hours under a nitrogen atmosphere.

After the reaction was completed, unreacted styrene and butylmethacrylate were removed from the reaction mixture using methanol. Then, the resultant was filtered and cleaned, and dried in a vacuum oven for 2 days, resulting in toner particles.

### <Comparative Example 6>

Toner particles were prepared by the same method as Comparative Example 1, except that the first composition and the second composition were mixed in a homogenizer.

According to Comparative Example 3, the conversion of the polymerization reaction was very low, and it was difficult to obtain spherical toner particles after the polymerization. Also, in the case when the first composition was prepared by using n-butyl alcohol (Comparative Example 4), the hydrophobic silica agglomerated, such that it was difficult to obtain a uniform first composition. Thus, the polymerization reaction to form the toner particles cold not be conducted.

Characteristics of the toner particles prepared by Example 1 and Comparative Examples 1, 2, 5, and 6 was evaluated as follows.

Particle diameters of the toner particles and particle diameter distribution were measured by a coulter counter or a laser particle diameter analyzer, and the surface of the toner particles was analyzed with a scanning electron microscope (SEM).

Dispersion properties of carbon black in the toner particles were evaluated with an optical microscope (Labophot-2, Nicon Co.), and represented as follows:
ⓞ : carbon black is very finely dispersed;
○ : carbon black is finely dispersed;
Δ : large particles of carbon black are slightly visible; and
× : large particles of carbon black are clearly visible.

The glass transition temperature was measured by using a differential scanning calorimeter (DSC), and the molecular weight was measured with a gel permeation chromatography (GPC).

The charge quantity of toner particles was measured by using a blow-off meter (Toshiba Co.).

On the other hand, the toner particles prepared by Example 1 and Comparative Examples 1, 2, 5 and 6 were measured to analyze the dispersion state of the carbon black, the average particle diameter, the glass transition temperature and the charge quantity. Their results are tabulated in Table 1.

**Table 1**

| classification | dispersion state of carbon black | average particle diameter (µm) | glass transition temperature (°C) | charge quantity (µc/g) |
|---|---|---|---|---|
| Comparative Example 1 | ○ | 12.57 | 68.04 | -11.54 |
| Comparative Example 2 | ○ | 13.76 | 66.14 | -12.16 |
| Example 1 | ⓞ | 12.87 | 64.37 | -15.48 |
| Comparative Example 5 | Δ | 38.28 | 65.36 | +7.35 |
| Comparative Example 6 | Δ | 26.99 | 66.12 | -9.56 |

As can be seen from Table 1, the toner particles prepared by Example 1 have excellent degree of dispersion compared with Comparative Examples 5 and 6.

Particularly, the diameter of the toner particles prepared by Comparative Example 5 tends to be divided into two classes, i.e., 20µm or more and 10µm or less. In this case, pigments are dispersed to some extent within the toner particles having 20µm or more in diameter while the pigment cannot be incorporated into the toner particles having 10µm or less in diameter.

Figures 1 through 3 are optical microscope photographs of the toner particles prepared by Comparative Example 1, Comparative Example 2 and Example 1 respectively, and Figures 4 and 5 are optical microscope photographs of the toner particles prepared by Comparative Examples 5 and 6.

Referring to Figures 1 through 3, it can be seen that the toner particles of Comparative Examples 1 and 2, and Example 1 have excellent degree of dispersion of the carbon black compared with Comparative Examples 5 and 6. In Particular, referring to Figure 3, in the case when cetyltrimethylammonium bromide (CTAB) is additionally added (Example 1), the carbon black is evenly dispersed into the toner particles.

Particle distribution of the toner particles prepared by Comparative Examples 1 and 2, Example 1 and Comparative Examples 5 and 6 are shown in Figures 6 to 10, respectively.

Referring to Figures 6 through 10, the distribution characteristics in particle diameter of the toner particles is improved in Comparative Examples 1 and 2 and Example 1, compared with Comparative Examples 5 and 6.

Also, as can be seen from Table 1, the toner particles prepared by Comparative Examples 1 and 2, and Example 1 show improvement in the charge quantity and the average particle diameter, compared with Comparative Examples 5 and 6.

Toner particles having improved in charge quantity, average particle diameter and particle diameter distribution can be prepared from the toner composition of embodiments of the present invention. Particularly, when the toner composition contains a surfactant, toner particles exhibiting improved dispersion properties of the colouring agent and charge controller can be obtained, thereby resulting in a better image quality.

## Claims

1. A toner polymerizable composition comprising a monomer for a binding resin, a colouring agent, a charge controller, a lubricant, a polymerization initiator, a stabilizer obtained by dispersing hydrophobic silica into distilled water of pH 10∼14, and then adjusting pH of the dispersion into 6∼8, and an ionic surfactant, and wherein the mixing ratio of the monomer for binding resin and the ionic surfactant is between 1000:1 and 2000:1 by weight.

2. The composition of claim 1, wherein the mixing ratio of the monomer for a binding resin and the silica solid content is between 50:1 and 25:1 by weight.

3. The composition of claim 1 or 2, wherein the ionic surfactant comprises a cationic surfactant.

4. The composition of any one of the preceding claims, wherein the ionic surfactant is selected from the group consisting of sodium lauryl sulfate, cetyltrimethylammonium bromide and cetyltrimethylammonium chloride.

5. A method of preparing a toner composition comprising the steps of:
(a) adjusting the pH of distilled water to pH 10∼14 with an aqueous base, and dispersing hydrophobic silica into the pH-adjusted distilled water;
(b) adjusting the pH of the mixture of the step (a) to pH 6∼8;
(c) mixing a monomer for a binding resin, a polymerization initiator, a charge controller, a lubricant a colouring agent and an ionic surfactant, and adding the mixture to the resultant of the step (b);
(d) preparing toner particles by polymerizing the resultant of the step (c); and
(e) removing foreign materials remaining on the surface of the toner particles;
wherein the mixing ratio of the monomer for binding resin and the ionic surfactant is between 1000:1 and 2000:1 by weight.

6. The method of claim 5, wherein the aqueous base is selected from the group consisting of ammonium hydroxide, sodium hydroxide and potassium hydroxide.

7. The method of claim 5, wherein the mixing ratio of the monomer for a binding resin and the silica solid content is between 50:1 and 25:1 by weight.

8. The method of any one of claims 5 to 7, wherein the ionic surfactant comprises a cationic surfactant.

9. The method of any one of claims 5 to 8, wherein the ionic surfactant is selected from the group consisting of sodium lauryl sulfate, cetyltrimethylammonium bromide and cetyltrimethylammonium chloride.

## Patentansprüche

1. Polymerisierbare Tonerzusammensetzung, umfassend ein Monomer für ein Bindeharz, ein Färbemittel, einen Ladungsregler, ein Gleitmittel, einen Polymerisationsinitiator, einen Stabilisator, erhalten durch Dispergieren von hydrophobem Siliciumdioxid in destilliertem Wasser von pH 10 ~ 14 und anschließendes Einstellen des pH der Dispersion auf 6 ~ 8, und einen ionischen oberflächenaktiven Stoff, und worin das Mischungsverhältnis des Monomers für das Bindeharz und des ionischen oberflächenaktiven Stoffs zwischen 1000 : 1 und 2000 : 1, bezogen auf das Gewicht, liegt.

2. Zusammensetzung nach Anspruch 1, worin das Mischungsverhältnis des Monomers für ein Bindeharz und des Gehalts von festem Siliciumdioxid zwischen 50 : 1 und 25 : 1, bezogen auf das Gewicht, liegt.

3. Zusammensetzung nach Anspruch 1 oder 2, worin der ionische oberflächenaktive Stoff einen kationischen oberflächenaktiven Stoff umfasst.

4. Zusammensetzung nach einem der vorhergehenden Ansprüche, worin der ionische oberflächenaktive Stoff ausgewählt ist aus der Gruppe bestehend aus Natriumlaurylsulfat, Cetyltrimethylammoniumbromid und Cetyltrimethylammoniumchlorid.

5. Verfahren zum Herstellen einer Tonerzusammensetzung, umfassend die Schritte:
(a) Einstellen des pH von destilliertem Wasser auf pH 10 ∼ 14 mit einer wässrigen Base und Dispergieren von hydrophilem Siliciumdioxid in dem pHeingestellten destillierten Wasser,
(b) Einstellen des pH der Mischung von Schritt (a) auf pH 6 ∼ 8,
(c) Vermischen eines Monomers für ein Bindeharz, eines Polymerisationsinitiators, eines Ladungsreglers, einer Gleitmittels, eines Färbemittels und eines ionischen oberflächenaktiven Stoffs und Zugeben der Mischung zu dem Produkt des Schritts (b),
(d) Herstellen von Tonerteilchen durch Polymerisieren des Produkts des Schritts (c) und
(e) Entfernen von auf der Oberfläche der Tonerteilchen zurückbleibenden Fremdmaterialien,
worin das Mischungsverhältnis des Monomers für das Bindeharz und des ionischen oberflächenaktiven Stoffs zwischen 1000 : 1 und 2000 : 1, bezogen auf das Gewicht, liegt.

6. Verfahren nach Anspruch 5, worin die wässrige Base ausgewählt ist aus der Gruppe bestehend aus Ammoniumhydroxid, Natriumhydroxid und Kaliumhydroxid.

7. Verfahren nach Anspruch 5, worin das Mischungsverhältnis des Monomers für ein Bindeharz und des Gehalts von festem Siliciumdioxid zwischen 50 : 1 und 25 : 1, bezogen auf das Gewicht, liegt.

8. Verfahren nach einem der Ansprüche 5 bis 7, worin der ionische oberflächenaktive Stoff einen kationischen oberflächenaktiven Stoff umfasst.

9. Verfahren nach einem der Ansprüche 5 bis 8, worin der ionische oberflächenaktive Stoff ausgewählt ist aus der Gruppe bestehend aus Natriumlaurylsulfat, Cetyltrimethylammoniumbromid und Cetyltrimethylammoniumchlorid.

## Revendications

1. Composition de toner polymérisable comprenant un monomère précurseur de résine de liant, un agent colorant, un contrôleur de charge, un lubrifiant, un amorceur de polymérisation, un stabilisant obtenu en dispersant de la silice hydrophobe dans de l'eau distillée de pH 10-14 et en ajustant ensuite le pH de la dispersion entre 6 et 8, et un agent tensio-actif ionique, et dans laquelle le rapport de mélange du monomère comme résine de liant et de l'agent tensio-actif ionique est entre 1000:1 et 2000:1 en poids.

2. Composition selon la revendication 1, dans laquelle le rapport de mélange du monomère précurseur de la résine de liant et de la teneur en silice solide est entre 50:1 et 25:1 en poids.

3. Composition selon la revendication 1 ou 2, dans laquelle l'agent tensio-actif ionique comprend un agent tensio-actif cationique.

4. Composition selon l'une quelconque des revendications précédentes, dans laquelle l'agent tensio-actif ionique est choisi dans le groupe constitué du laurylsulfate de sodium, bromure de cétyltriméthylammonium et chlorure de cétyltriméthylammonium.

5. Procédé de préparation d'une composition de toner comprenant les étapes consistant à :
(a) ajuster le pH d'eau distillée à pH 10-14 avec une base aqueuse, et disperser de la silice hydrophobe dans l'eau distillée ajustée en pH ;
(b) ajuster le pH du mélange de l'étape (a) à pH 6-8 ;
(c) mélanger le monomère précurseur de la résine de liant, l'amorceur de polymérisation, le contrôleur de charge, le lubrifiant, l'agent colorant et l'agent tensio-actif ionique, et ajouter le mélange au résultat de l'étape (b) ;
(d) préparer des particules de toner en polymérisant le résultat de l'étape (c) ; et
(e) éliminer les matériaux étrangers restant sur la surface des particules de toner ;
dans lequel le rapport de mélange du monomère précurseur de la résine de liant et l'agent tensio-actif ionique est entre 1000:1 et 2000:1 en poids.

6. Procédé selon la revendication 5, dans lequel on choisit la base aqueuse dans le groupe constitué de l'hydroxyde d'ammonium, l'hydroxyde de sodium et l'hydroxyde de potassium.

7. Procédé selon la revendication 5, dans lequel le rapport de mélange du monomère précurseur de la résine de liant et la teneur en silice solide est entre 50:1 et 25:1 en poids.

8. Procédé selon l'une quelconque des revendications 5 à 7, dans lequel l'agent tensio-actif ionique comprend un agent tensio-actif cationique.

9. Procédé selon l'une quelconque des revendications 5 à 8, dans lequel l'agent tensio-actif ionique est choisi dans le groupe constitué du laurylsulfate de sodium, bromure de cétyltriméthylammonium et chlorure de cétyltriméthylammonium.
